

1,376,403.

R. G. COATES.  
INGOT MOLD AND METHOD OF MAKING SAME,  
APPLICATION FILED NOV. 13, 1918.

Patented May 3, 1921.



Fig. 1.

Fig. 2.



13 Ray G. Coates  
Inventor  
George F. Murray  
Attorney

# UNITED STATES PATENT OFFICE.

RAY G. COATES, OF PASADENA, CALIFORNIA, ASSIGNOR TO VALLEY MOULD AND IRON CORPORATION, OF SHARPSVILLE, PENNSYLVANIA, A CORPORATION OF NEW YORK.

## INGOT-MOLD AND METHOD OF MAKING SAME.

1,376,403.

Specification of Letters Patent.

Patented May 3, 1921.

Application filed November 12, 1918. Serial No. 262,279.

To all whom it may concern:

Be it known that I, RAY G. COATES, a citizen of the United States, and a resident of the city of Pasadena, in the county of Los Angeles, State of California, have invented new and useful Improvements in Ingot-Molds and Methods of Making Same, of which the following is a specification.

This invention relates broadly to metallurgy, more specifically to an ingot mold and the method of making the same.

The principal object of the present invention is a lugged ingot mold of direct metal, that is iron directly from the blast furnace, and wherein the lugs and head of the mold are of increased strength and both the top and bottom of the mold are of a smooth finish.

An equally important and primary object of the present invention is the method for producing the above specified ingot mold, which method comprises casting the ingot mold in inverted position with the lugs near the bottom of the sand mold in which the ingot mold is cast.

This invention possesses many other advantageous features, some of which, together with the foregoing, will be set out more at length in the following description wherein will be outlined in full that form of the invention which I have selected for an illustration in the drawings accompanying and forming a part of the present specification.

In the drawings and specification I have described only the preferred form of my generic invention, but it is to be understood that I do not limit myself to such form because my invention may be embodied in a multiplicity of forms each being a species of my invention. It being understood that by the claims succeeding the description of my invention I desire to cover the invention in whatsoever form it may be embodied or practised.

Figure 1 is a sectional view through the sand mold which may be used in carrying out my invention.

Fig. 2 is a sectional view through the sand mold taken at substantially right angles to the section shown in Fig. 1, and illustrating the arrangement for pouring or casting in carrying out my invention.

Fig. 3 is a perspective view of an ingot mold in accordance with my invention.

Heretofore in the art it has been the practice to cast ingot molds, used for making steel ingots, by casting these molds upright from direct metal or cupola iron. Direct metal (blast furnace metal) is better suited for ingot molds than is cupola iron for the reason that blast furnace metal will stand more "heats" before becoming useless than will molds made from cupola metal. Direct metal or blast furnace metal, such as is usually made into pig iron, throws off a large amount of graphite or free carbon when cast into molds. When the molten iron from the blast furnace slowly cools, carbon is released as "graphite" and a part rises to the surface through the still fluid iron, just as particles of cork would rise through water. A certain portion of very light graphite, which is completely released from the molten iron, is caught by the strong convective currents of air that always rise above the molten iron, and floats off through the air to be deposited by gravity elsewhere in the foundry. A larger portion of the graphite, however, does not leave the surface of the metal but accumulates upon, and in, the upper strata of metal so that this portion of the metal is apt to be porous or, to use a term in the art, is "rotten."

This accumulation of excess free carbon is more or less adjacent the surface of the molten metal and does not extend in like proportion downward through the body of a relatively deep mass of molten metal. The longer the metal remains in fluid condition, the greater the opportunity for the freed carbon to rise.

In view of the tendency to release free carbon, it is desirable that any large casting such as ingot molds from direct metal shall be done in open molds, because if a cover or "cope" be placed over the mold to form a finished top to the casting, the graphite will be trapped on the top of the casting and will accumulate to a greater extent than if the top were cast open. It is, therefore, customary in making ingot molds to cast from direct metal in open molds and attempt to remove accumulated graphite by raking off or skimming the mold when it is nearly filled, and then to fill the mold to its final height. After the casting has cooled somewhat, but while it is still hot, a hole is broken into the "shrinkage pipe" adjacent the surface of the casting and fresh hot metal is

poured into this hole so as to fill the shrinkage pipe as much as possible. This refilling of the shrinkage pipe from the ladle, in substantially all cases, is accompanied by an undesirable flow of metal that spreads over the top of the mold, thereby making a bad end on the final casting and more or less injuring the mold.

Ingot molds, in the most common form, 10 are provided with lugs adjacent the upper end of the ingot mold to enable the ingot mold to be withdrawn from the steel ingot which may be cast therein. When such type of ingot molds is made from direct or 15 blast furnace metal, it has been found that the rising graphite frequently accumulates in the cavities that form the lugs on the finished ingot mold, and thereby prevents the free flow of iron into these cavities so 20 that the lugs of the casting are porous and weak. Ingot molds are frequently made with top staples extending from the mold and where such top staples are set in the casting mold to be cast in the casting, they 25 interfere with the process of raking off the top of the metal and they are liable to be moved out of place during the raking off and generally add complications to an already difficult problem. Because of eco- 30 nomic reasons it is essential that hand work on ingot molds be reduced to a minimum, and yet, it is very desirable that the tops of these molds shall be relatively smooth, because it is much easier in practice to keep a 35 smooth top clean from splashed steel and drippings from the ladle, and the smooth top is much more easily capped when "wild" metal is poured into the mold. Since the joint between the cap and the smooth top 40 being closer than where the top is rough, it forms a thinner and more equal "fin", which more certainly chills and closes the joint between the top and the cap, the latter being held down by a wedge placed under the top 45 staples and over the cap.

My invention comprises an ingot mold cast from direct metal, also includes the process or method by which such an ingot mold is produced. In carrying out my 50 process, the ingot mold is cast in a reverse or up-side-down position in a sand mold with the lugs of the ingot mold near the bottom of the sand mold, and the end of the mouth of the ingot mold adjacent the bottom plate. Since the larger portion of the metal in the mold will be above the position of the lugs, it follows that the larger part of the floating or completely freed graphite will separate out from the iron above the 55 lug position and, therefore, there is less opportunity for such graphite to accumulate in the lug cavities and obviously there is a less amount of graphite to be accumulated. The ferrostatic pressure of the metal in this 60 part of the mold is much greater than that

adjacent the upper end of the mold and, therefore, the lug cavities of the sand mold are completely filled with sound metal. The rising floating graphite meets no obstructions in its path to the surface of the iron 70 and, consequently, it freely accumulates on the surface at the top of the casting and may be raked off or not as is desired. By casting the ingot mold in inverted position, the bottom plate of the sand mold may be 75 provided with cavities in which staples may be set in sand so that the surface of the casting is free from obstruction and the accumulated graphite may be very easily removed by raking as specified. It is preferable that the casting for the ingot mold shall be made somewhat longer than the length of the finished ingot mold. This feature forms a sink head portion around the entire top of the casting so that the 80 pipe, tending to form in the cooling of the metal, will be fed from a relatively large area and shrinkage will be from as large a surface as is possible and for as little vertical height, in the casting, as is possible. 85 When the cast ingot mold is taken from the sand, the extra length is cut off by a saw or other tool and the "rotten" portion, due to excessive graphite as well as the shrinkage cavities, is in the cut-off piece. This 90 cut-off piece is practically pig iron and salable as such.

This process, it will be seen, provides that the base of the body of the ingot mold shall be a finished base, therefore, it forms a good 100 joint with the "stool" on which the mold is intended to be set and used to mold ingots, and also the top of the mold is smooth because it has been cast against the bottom plate and sand, and the lugs being cast under 105 good ferrostatic head from clean metal, are sound throughout. This ingot mold, it will be seen, really is as well finished a mold as is ordinarily cast from cupola metal, and at the same time possesses more desirable 110 metallurgical qualities because of being cast from direct metal and at the same time is more economical in manufacture. That part of the metal designed to be cut off may form a direct continuation of the body of 115 the ingot mold itself or it may be made larger to give a larger surface area and to comprise a lateral projection on the top end of the casting to comprise a hold for grab hooks for lifting the casting up for the sawing-off operation. In the latter case the upper edge of the sand mold may be rounded off and, therefore, be somewhat more durable than if left, as is usual, with the straight corner. In this practice the amount of 120 metal cast for this extension to be cut off may be no more than if the area of the extension were not enlarged, for it may be slightly shorter to make up for the metal used in 125 forming the projection.

In the preferred form of carrying out my invention, the mold in which my ingot mold is cast comprises a bottom piece 1 which preferably is made of iron and is provided with sand cavities 2 in which lugs or staples 4 are adapted to be set-in or embedded with the ends of the staples extending upwardly in such manner as to be cast-in in the ingot mold when this mold is made. The sand mold, for the ingot mold, preferably is made in two or more parts and comprises a flask 5 of iron in which molding sand 6 has been tamped around the pattern for the ingot mold which is positioned in such manner that the ingot mold is inverted with the lugs 7 adjacent the bottom of the flask and the extreme end of the mold is in contact with the bottom plate so it results that this portion of the ingot mold is slightly chilled. The interior of the ingot mold is preferably formed by an iron core 12 which is covered with sand in order that the core may be easily withdrawn and to keep the iron core from chilling the inner surface of the mold. Preferably this flask mold is made longer than the finished length of the ingot mold in order that the upper portion of the flask mold may comprise a cavity in which graphite and the shrinkage cavities may collect and form for the reasons specified.

Fig. 2 is a section taken at substantially right angles to the section shown in Fig. 1, and more clearly illustrates the specific manner in which the ingot mold is cast in that the metal is poured through a runner 8, the bottom of which is provided with a small cavity 9 adjacent the bottom plate 1, and the first metal flowing into the mold will close all cracks with "fins" so that when the ferrostatic pressures increase the cracks will be sealed and the metal will be contained entirely within the mold section proper. A larger upper conduit or gate 10 is provided between the runner 8 and the interior of the sand mold so that when the heavier head of metal is poured it flows through this larger gate 10 and gradually fills the mold section. It will be noted that in the process of casting in this mold the metal rises upwardly in the same direction as is the travel of the graphite above referred to; so therefore it will be seen that the movement of the graphite is facilitated by this process and I am enabled to cast a clear, strong ingot mold.

The upper end of the runner 8 is provided with a pouring funnel 11 made of sand and clay. This obviates splashing of metal over into the mold cavity proper. When the casting is cooled, the metal in the runner is cut off.

Referring now more particularly to Fig. 3 which illustrates an ingot mold made according to my invention, the portion 13 indicated by dotted lines represents that part of the ingot mold casting which was formed in

the upper part of the sand mold and which has been cut away by a metal saw or other suitable tool. As previously stated, this cut-off material is substantially the same as pig iron and is salable as such. 70

Having described my invention, what I claim is:—

1. As an article of manufacture a lugged ingot mold of direct blast furnace metal and having a body portion with a squarely 75 cut base, and having lugs adjacent the mouth of the body portion, the metal forming the lugs and mouth of said ingot mold being integral with the body of the mold and of the toughest and most dense metal 80 in the said ingot mold, and with more free carbon in the metal at the base of the mold than at the mouth thereof.

2. As an article of manufacture an ingot mold of direct blast furnace metal having a 85 body portion with a base finished square with the axis of the mold, and with said body portion provided with lugs adjacent the mouth of the ingot mold, and said mouth being integral with the body portion 90 and comprising a smooth chilled finished portion when the ingot mold is taken from the sand mold, with the metal forming the mouth of the mold being substantially free of graphite. 95

3. The method of manufacturing ingot molds from direct blast furnace metal, which comprises providing a sand mold having the recesses for the lugs on the ingot mold arranged in the bottom side walls of the said sand mold, then introducing the direct metal into the lower portion of the sand mold whereby the molten metal in the sand mold rises in the same direction as the graphite which is freed during the cooling 105 of the molten metal. 100

4. The method of manufacturing ingot molds from direct blast furnace metal, which method comprises providing a sand mold with recesses for the lugs of the ingot 110 mold and arranged adjacent the bottom of the sand mold, providing a bottom plate for the bottom of the sand mold; then introducing the direct metal into the sand mold adjacent the bottom thereof in such manner 115 that the portion of metal forming the mouth and lugs of the ingot mold is at all times under the greatest ferrostatic pressure and is continually fed with fresh metal during the casting operation. 120

5. The method of manufacturing ingot molds from direct blast furnace metal, which method comprises providing a sand mold with matrix of the ingot mold arranged in the sand mold in inverted position and having the lug-forming recesses adjacent the bottom of the said sand mold, then filling the said sand mold by direct metal introduced through a gate adjacent the bottom of the sand mold. 125 130

6. The method of manufacturing ingot  
molds from direct metal which method com-  
prises casting the ingot mold in inverted po-  
sition with the lugs thereof at the bottom of  
5 the casting mold, providing a vertical height  
to the casting which is greater than the  
length required for the finished ingot mold;  
then cutting off that portion of the casting  
in which are located the shrinkage pipes  
10 and accumulated graphite.

7. The method of manufacturing ingot  
molds from direct metal, which method

comprises providing a sand mold in which  
the matrix for the ingot mold is inverted  
and with the lugs at the bottom of the sand 15  
mold, then introducing the direct metal into  
the sand mold in such manner that the direc-  
tion of movement of the molten metal in the  
sand mold is the same as the direction of  
movement of freed carbon; then cutting off 20  
from the casting that portion containing  
accumulated carbon and shrinkage pipes.

RAY G. COATES.